

3,223,634

## LUBRICANT COMPOSITIONS

David X. Klein, Upper Montclair, N.J., assignor, by  
mesne assignments, to Texaco Chemicals, Inc., a cor-  
poration of Delaware  
No Drawing. Filed May 28, 1963, Ser. No. 283,693  
15 Claims. (Cl. 252—42.7)

This invention relates to synthetic ester fluids which are  
resistant to oxidation at elevated temperatures and more  
particularly to ester lubricant compositions which are  
useful as lubricants in jet aircraft engines.

Jet aircraft engines require a lubricant which provides  
the necessary lubricity to minimize the friction and which  
meets the other requirements with respect to viscosity,  
thermal stability, fire point, pour point, and the like. The  
design of more powerful jet engines has led to an in-  
crease in the temperatures under which the lubricant is  
used. For example, a high temperature lubricant should  
be stable under oxidative conditions at temperatures above  
400° F.

Esters of aliphatic acids and polyols are useful as lub-  
ricants at elevated temperatures. However, these esters  
are not sufficiently stable under oxidative conditions at  
temperatures in the order of 400° F. over extended  
periods. Under such conditions the esters sludge badly,  
build up viscosity, and develop high acidity which causes  
severe corrosion.

It has been discovered that a lubricant comprising as  
the base fluid a major proportion of a polyol ester and  
a minor proportion each of a diaromatic secondary amine  
and a metal chelate of a salicylimine or 5-nitrosalicylimine  
has excellent stability under oxidative conditions at ele-  
vated temperatures.

The polyol esters are esters of a single or a mixture of  
polyols and a single or a mixture of saturated, straight  
or branched chain, monocarboxylic aliphatic acids. Al-  
ternatively saturated, aliphatic dicarboxylic acids may be  
used as part of the esterification acids. The anhydrides of  
the monocarboxylic or dicarboxylic acids may be used  
and are equivalents.

The preferred polyols are the neopentyl alcohols con-  
taining from 2 to 4 methylol groups although other al-  
cohols containing from 2 to 4 hydroxyl groups may be  
used as is known in the prior art. Among the preferred  
polyols are trimethylethane, trimethylolpropane, tri-  
methylolbutane, pentaerythritol, neopentyl glycol, 2-butyl-  
2-ethyl-1,3-propanediol, and 2,2,4-trimethyl-1,3-pentane-  
diol.

The saturated monocarboxylic acids may contain from  
2 to 18 carbons depending in part on the polyol but pri-  
marily on the viscosity requirements and to a certain  
extent on whether or not mixtures of acids are used.  
In general, acids containing 12 or more carbon atoms  
produce esters which are solids at room temperature al-  
though this can be overcome in part by the use of a  
mixture of such a long chain acid with a short chain  
acid. Particularly for base fluids which must also be  
fluid at room temperature and preferably have a pour  
point of —40° F. or less, better results are obtained with  
acids containing from 4 to 10 carbon atoms. The pre-  
ferred acids are those containing from 5 to 9 carbon  
atoms with optimum results being obtained with a single  
acid or a mixture of acids containing an average of  
from 5 to 8 carbon atoms.

When a dicarboxylic, saturated aliphatic acid is used,  
the amount used of such acid is one mole of acid per  
two moles of polyol to produce an ester of the formula,  
R—acid—R, where R represents the alcohol moiety.  
The remaining hydroxyl groups of the alcohol are es-  
terified with the monocarboxylic acids previously de-

scribed. The dibasic acids are saturated aliphatic acids  
and they may contain from 3 to 36 carbon atoms in their  
formula. The preferred acids are sebacic acid, azelaic  
acid, and adipic acid. However, the present invention is  
not limited to these acids and mixtures of such acids, for  
example, a mixture of sebacic and adipic acids, may be  
used. Illustrative esters are disclosed in United States  
Patent No. 3,048,608 and British Patent No. 915,161,  
published January 9, 1963.

The following esters are illustrative of those which may  
be used as the base fluid; however, it is to be under-  
stood that these are not the only esters which may be  
used: trimethylolpropane divalerate monopalargonate, tri-  
methylolpropane monovalerate monocaproate monocap-  
rylate, trimethylolpropane divalerate monoheptanoate,  
trimethylolpropane dibutyrate monopalargonate, trimeth-  
ylethane divalerate monopalargonate, trimethylethane  
dicaproate monocaprylate, trimethylethane dibutyrate  
monopalargonate, bis (neopentyl glycol monopalargonate)  
azelate, bis (pentaerythritol trivalerate) adipate, bis (pen-  
taerythritol tricaproate) sebacate, pentaerythritol tetra-  
caproate, and pentaerythritol dicaproate divalerate.

The preparation of such esters is known and any  
suitable procedure may be followed. Preferably the  
polyol esters are prepared by the esterification of the polyol  
in the presence of a slight excess of the monocarboxylic  
acid to promote the production of esters substantially free  
of hydroxyl groups. If a dicarboxylic acid is used, it  
is used in an amount equal to one mole of acid per  
two moles of polyol, and the dicarboxylic acid may be  
reacted with the polyol prior to or at the same time as  
the monocarboxylic acid. The esterification may be  
carried out, for example, at temperatures in the range of  
about 180°—240° C. Water is removed preferably but  
not necessarily in the presence of an azeotropic agent  
such as a liquid hydrocarbon. Any unreacted acid should  
be removed. The preparation of such esters is disclosed  
in United States Patent No. 3,036,005 and in the A.C.S.  
Monograph No. 136 ("The Pentaerythrins"; Berlow,  
Barth, and Snow; 1958).

The diaromatic secondary amines include diaryl amines,  
aryl-alkaryl amines and dialkaryl amines, with the aryl  
groups preferably having no more than 5 benzene rings  
and the alkyl substituents, when present, having no more  
than 24 carbon atoms. Among the specific diaromatic  
secondary amines which may be used are phenyl- $\alpha$ -  
naphthylamine, p,p'-diocetylphenylamine, and phenyl- $\beta$ -  
naphthylamine.

The metal chelates may be prepared from salicylalde-  
hyde or 5-nitro-salicylaldehyde, an amine and the metal  
as the chloride, in the manner described in Shrine and  
Fuson, "Systematic Identification of Organic Com-  
pounds," 4th edition, page 112. The reactions involved  
may be represented by the following equation:



wherein Y represents  $\text{NO}_2$  or H; M represents Ni, Co, or Zn; and R represents



or



and X represents H,  $\text{CH}_3$ , or Cl. Illustrative metal are those prepared from the following materials:

| Aldehyde               | Amine                    | Metal   |
|------------------------|--------------------------|---------|
| 5-Nitrosalicylaldehyde | Aniline                  | Nickel. |
| 5-Nitrosalicylaldehyde | p-Phenoxy aniline        | Do.     |
| Salicylaldehyde        | Aniline                  | Do.     |
| 5-Nitrosalicylaldehyde | Aniline                  | Zinc.   |
| 5-Nitrosalicylaldehyde | p-Phenoxyphenoxy aniline | Nickel. |
| 5-Nitrosalicylaldehyde | o-Toluidine              | Do.     |
| 5-Nitrosalicylaldehyde | o-Chloroaniline          | Do.     |
| 5-Nitrosalicylaldehyde | 2-Ethylhexylamine        | Do.     |
| 5-Nitrosalicylaldehyde | Aniline                  | Cobalt. |

Mixtures of these chelates may be used and may be preferred. For example, a mixture may be used comprising equal or unequal portions of nickel bis (N-phenyl-5-nitrosalicylimine) and nickel bis (N-phenyl-salicylimine).

#### Example 1

The preparation of trimethylolpropane divalerate monopalargonate may be carried out as follows: a mixture of 268 grams (2.0 moles) of trimethylolpropane, 490.3 grams (4.8 moles) of valeric acid, 379.8 grams (2.4 moles) of pelargonic acid, 110.5 grams of xylene, and

15

20

25

30

35

60

65

70

75

are representative of trimethylolpropane divalerate monopalargonate prepared by this procedure.

|                                  |              |
|----------------------------------|--------------|
| Acid number                      | 0.028        |
| Hydroxyl content                 | percent 0.08 |
| Saponification value             | 378.8        |
| Flash point                      | ° F. 435     |
| Pour point                       | ° F. -92     |
| Viscosity (centistokes):         |              |
| at 210° F.                       | 3.39         |
| at 100° F.                       | 14.30        |
| at -65° F.                       | 12,830       |
| Viscosity index (Dean and Davis) | 127.4        |

#### Example 2

Polyol esters of trimethylolpropane divalerate monopalargonate prepared in the manner described in Example 1 were subjected to oxidation tests with and without various additives. These tests were performed using a 20 ml. portion maintained at 425° F. for 24 hours with 20 liters per hour of dry air flow through the fluid. In each instance the viscosity and acid number were determined prior to the test. After the test the amount of fluid lost was determined as was the viscosity and acid number and the percent change in viscosity at 100° F. was calculated. Each test was run in replicate. The compositions tested were (1) polyol ester base fluid with no additive, (2) polyol ester base fluid containing 1% by weight of phenyl- $\alpha$ -naphthylamine and 1% by weight of nickel bis (N-phenyl-5-nitrosalicylimine), (3) polyol ester base fluid containing 1% by weight of nickel bis (N-phenyl-5-nitrosalicylimine) alone, and (4) polyol base fluid containing 1% by weight of N-ethylphenodiphenyl silazine. The last mentioned combination is described in U.S. Patent No. 3,036,005. The foregoing percentages of additives are based on the weight of the polyol ester.

TABLE I

| Fluid                                                                                                                                | Before Test                        |             |                    | After Test                         |                                     |             | Remarks                                 |
|--------------------------------------------------------------------------------------------------------------------------------------|------------------------------------|-------------|--------------------|------------------------------------|-------------------------------------|-------------|-----------------------------------------|
|                                                                                                                                      | Viscosity (centistokes) at 100° F. | Acid Number | Percent Fluid Loss | Viscosity (centistokes) at 100° F. | Percent Viscosity Change at 100° F. | Acid Number |                                         |
| Base fluid, no additive                                                                                                              | 14.85                              | 0.2         | 33.2               | 513.4                              | 3,346.                              | 16.6        | Darkened badly, no insolubles.          |
| Replicate                                                                                                                            | 14.85                              | 0.2         | 32.7               | 460.9                              | 2,993.                              | 13.6        | Do.                                     |
| Base fluid containing 1% by weight of phenyl- $\alpha$ -naphthylamine and 1% by weight of nickel bis (N-phenyl-5-nitrosalicylimine). | 15.50                              | 0.3         | 3.8                | 16.59                              | 7.03                                | 0.1         | Darkened; negligible insolubles.        |
| Replicate                                                                                                                            | 15.50                              | 0.3         | 6.1                | 16.70                              | 7.74                                | 0.1         | Do.                                     |
| Base fluid containing 1% by weight of nickel bis (N-phenyl-5-nitrosalicylimine).                                                     | 15.23                              | 0.2         | 26.3               | 343.2                              | 2,153.                              | 14.7        | Darkened; moderate insoluble formation. |
| Replicate                                                                                                                            | 15.23                              | 0.2         | 22.0               | 185.5                              | 1,118.                              | 15.6        | Do.                                     |
| Base fluid containing 1% by weight of phenyl- $\alpha$ -naphthylamine and 1% by weight of N-ethyl-phenodiphenyl silazine.            | 15.60                              | 0.3         | 6.4                | 17.47                              | 12.0                                | 0.4         | Darkened; no insolubles.                |
| Replicate                                                                                                                            | 15.60                              | 0.3         | 6.5                | 17.69                              | 13.4                                | 0.5         | Do.                                     |

22.1 grams of activated carbon is heated to 175°-180° C. in two hours and maintained at this temperature for about 23 hours. At the end of this time the reaction mixture has an acid number of 42.3. After sparging with carbon dioxide to remove the xylene, the reaction mixture is cooled to 100° C. and filtered to remove the carbon. The crude ester is then diluted with its own volume of petroleum ether. The crude ester solution is washed with sufficient 5% aqueous sodium hydroxide solution to neutralize the unreacted acid and then with 12% sodium chloride solution until neutral. After the addition of about 2% by weight of activated carbon, the solution is heated at about 40° C. at about 20 mm. absolute pressure and then at 160°-180° C. at 2 mm. absolute pressure to remove the water, petroleum ether, and any other low boiling materials that may be present. The residue is cooled to 100° C. and filtered. The following properties

60

65

70

75

#### Example 3

The ester base fluid of Example 1 containing additives was subjected to wear tests in a "precision-Shell four ball extreme pressure tester." This test is described in the literature. Briefly stated, the tester comprises a holder for holding three lower balls in fixed positions. An upper ball is pressed against the lower fixed balls under a predetermined load and rotated while the three points of contact are lubricated with the lubricant under test. The diameters of the three load scars on the lower balls are measured. In this example two lubricants were subjected to comparative tests. In one series of tests, the upper ball was rotated at 1200 r.p.m. for two hours at 167° F. In a second series of tests, the upper ball was rotated at 600 r.p.m. for two hours at 400° F. In each series of tests two somewhat different groups of balls were

used. One group was of mild steel and the other group was of stainless steel. The loads applied were 10 kilograms and 40 kilograms, respectively. At the end of each test the diameter of the scar on each of the three lower balls was measured both vertically and horizontally and the average of the six measurements in millimeters is the value used for the scar diameter in describing the results.

Lubricant composition A was the base fluid containing 1% by weight of phenyl- $\alpha$ -naphthylamine and 1% by weight of N-ethylphenodiphenyl silazine. The second composition, composition B, was the base fluid containing 1% by weight of phenyl- $\alpha$ -naphthylamine and 0.8% by weight of nickel bis (N-phenyl-5-nitrosalicylimine). In preparing composition B, 1% of the chelate was added. The composition was filtered and undissolved chelate removed, leaving 0.8% chelate in the lubricant.

TABLE II

| Fluid              | 600 r.p.m., 2 hours, 400° F. |        |                       |         |
|--------------------|------------------------------|--------|-----------------------|---------|
|                    | Mild Steel Balls             |        | Stainless Steel Balls |         |
|                    | 10 Kg.                       | 40 Kg. | 10 Kg.                | 40 Kg.  |
| Composition A:     |                              |        |                       |         |
| Scar diameter..... | 0.742                        | 1.068  | 0.454                 | 1.0.835 |
| Oil change.....    | (2)                          | (2)    | (2)                   | (2)     |
| Composition B:     |                              |        |                       |         |
| Scar diameter..... | 0.371                        | 0.884  | 0.475                 | 0.683   |
| Oil change.....    | (2)                          | (2)    | (2)                   | (2)     |

  

| Fluid              | 1200 r.p.m., 2 hours, 167° F. |        |                       |         |
|--------------------|-------------------------------|--------|-----------------------|---------|
|                    | Mild Steel Balls              |        | Stainless Steel Balls |         |
|                    | 10 Kg.                        | 40 Kg. | 10 Kg.                | 40 Kg.  |
| Composition A:     |                               |        |                       |         |
| Scar diameter..... | 0.681                         | 0.864  | 0.444                 | 0.876   |
| Oil change.....    | (3)                           | (3)    | (3)                   | (3)     |
| Composition B:     |                               |        |                       |         |
| Scar diameter..... | 0.510                         | 0.787  | 0.508                 | 1.0.824 |
| Oil change.....    | (3)                           | (3)    | (3)                   | (3)     |

### NOTE:

1 Wear scar is rough.

2 Oil darkened.

<sup>3</sup> No change in oil color.

Scar diameter = Average of six measurements.

The present combination of additives in lubricant B compares favorably with the previously known combination of additives in lubricant A. This known combination is one of the best anti-oxidants available up to this time for high temperature synthetic ester lubricants and was used for comparative purposes for this reason.

The diaromatic secondary amine and the metal chelate each will be used normally in an amount in the range of from 0.25% to 3% by weight of the polyol ester and preferably in an amount in the range of from 0.5% to 2% by weight of the polyol ester. However, the present invention is not limited to these amounts and larger amounts may be used although such larger amounts will be a minor amount based on the weight of the polyol esters. These two materials may be added separately to the polyol ester or may be pre-mixed for subsequent use.

A mixture of metal chelates may be used and may be preferred as, in general, the chelates prepared from salicylaldehyde increase the solubility of the chelates prepared from 5-nitro-salicylaldehyde. Mixtures of these two aldehydes may be used in preparing the chelates. Also, a mixture of amines, for example, a mixture of aniline and p-phenoxyaniline, may be used in preparing the chelates.

The lubricant compositions also may contain other additives such as detergents, pour point depressants, viscosity index improvers, etc. The base fluid need not 75

consist of the polyol ester and may include other lubricants.

I claim:

1. A lubricant composition comprising an aliphatic acid ester of a polyol containing from 2 to 4 hydroxyl groups, said acid being selected from the group consisting of (1) saturated, aliphatic monocarboxylic acids and (2) at least one saturated, aliphatic monocarboxylic acid and at least one saturated, aliphatic dicarboxylic acid, said ester being stabilized against oxidative degradation by a minor amount relative the amount of ester of a diaromatic secondary amine selected from the group consisting of diaryl amines, aryl alkaryl amines and dialkaryl amines, and a minor amount relative the amount of ester of metal chelate represented by the formula:



25 wherein Y represents a member selected from the group consisting of  $\text{NO}_2$  and H; M represents a member selected from the group consisting of Ni, Co, and Zn; R represents a member selected from the group consisting of



25 and



and X represents a member selected from the group consisting of H,  $\text{CH}_3$ , and Cl.

2. A lubricant composition comprising an acid ester of a neopentyl alcohol containing from 2 to 4 methylol groups, said acid being selected from the group consisting of (1) saturated, aliphatic monocarboxylic acids and (2) 45 at least one saturated, aliphatic monocarboxylic acid and at least one saturated, aliphatic dicarboxylic acid, said ester being stabilized against oxidative degradation by from 0.25% to 3% by weight of a diaromatic secondary amine selected from the group consisting of diaryl amines, 50 aryl alkaryl amines and dialkaryl amines, and from 0.25% to 3% by weight of metal chelate represented by the formula:



wherein Y represents a member selected from the group consisting of  $\text{NO}_2$  and H; M represents a member selected from the group consisting of Ni, Co, and Zn; R represents a member selected from the group consisting of



and



and X represents a member selected from the group consisting of H, CH<sub>3</sub>, and Cl.

3. A lubricant composition comprising an acid ester of a neopentyl alcohol containing from 2 to 4 methylol groups, said acid being saturated, aliphatic monocarboxylic acid containing from 4 to 10 carbon atoms, said ester being stabilized against oxidative degradation by a minor amount based on the amount of ester of a diaromatic secondary amine selected from the group consisting of diaryl amines, aryl alkaryl amines and dialkaryl amines, and a minor amount based on the amount of ester of metal chelate represented by the formula:



wherein Y represents a member selected from the group consisting of NO<sub>2</sub> and H; M represents a member selected from the group consisting of Ni, Co, and Zn; R represents a member selected from the group consisting of



and



and X represents a member selected from the group consisting of H, CH<sub>3</sub>, and Cl.

4. A lubricant comprising a major proportion of an acid ester of a neopentyl alcohol containing from 2 to 4 methylol groups, said acid being a mixture of saturated, aliphatic monocarboxylic acids containing an average of from 5 to 8 carbon atoms, said ester being stabilized against oxidative degradation by a minor amount based on the amount of ester of a diaromatic secondary amine selected from the group consisting of diaryl amines, aryl alkaryl amines and dialkaryl amines, and a minor amount based on the amount of ester of metal chelate represented by the formula:



wherein Y represents a member selected from the group consisting of NO<sub>2</sub> and H; M represents a member selected from the group consisting of Ni, Co, and Zn; R represents a member selected from the group consisting of



and



and X represents a member selected from the group consisting of H, CH<sub>3</sub>, and Cl.

5. A lubricant comprising a major proportion of an aliphatic acid ester of a polyol containing from 2 to 4

hydroxyl groups, said acid being selected from the group consisting of (1) saturated, aliphatic monocarboxylic acids, and (2) at least one saturated, aliphatic monocarboxylic acid and at least one saturated, aliphatic dicarboxylic acid, said ester being stabilized against oxidative degradation by a minor amount based on the amount of ester of phenyl- $\alpha$ -naphthylamine, and a minor amount based on the amount of ester of nickel bis (N-phenyl-5-nitrosalicylimine).

10. 6. A lubricant comprising a major proportion of an acid ester of a neopentyl alcohol containing from 2 to 4 methylol groups, said acid being saturated, aliphatic monocarboxylic acid containing from 4 to 10 carbon atoms, said ester being stabilized against oxidative degradation by a minor amount based on the amount of ester of phenyl- $\alpha$ -naphthylamine, and a minor amount based on the amount of ester of nickel bis (N-phenyl-5-nitrosalicylimine).

15. 7. A lubricant comprising a major proportion of an acid ester of trimethylolethane, said acid being saturated, aliphatic monocarboxylic acid containing from 4 to 10 carbon atoms, said ester being stabilized against oxidative degradation by a minor amount based on the amount of ester of phenyl- $\alpha$ -naphthylamine, and a minor amount based on the amount of ester of nickel bis (N-phenyl-5-nitrosalicylimine).

20. 8. A lubricant comprising a major proportion of an acid ester of trimethylopropane, said acid being saturated, aliphatic monocarboxylic acid containing from 4 to 10 carbon atoms, said ester being stabilized against oxidative degradation by from 0.25% to 3% by weight of phenyl- $\alpha$ -naphthylamine, and from 0.25% to 3% by weight of nickel bis (N-phenyl-5-nitrosalicylimine).

25. 9. A lubricant comprising a major proportion of an acid ester of pentaerythritol, said acid being saturated, aliphatic monocarboxylic acid containing from 4 to 10 carbon atoms, said ester being stabilized against oxidative degradation by from 0.25% to 3% by weight of phenyl- $\alpha$ -naphthylamine, and from 0.25% to 3% by weight of nickel bis (N-phenyl-5-nitrosalicylimine).

30. 10. A lubricant composition comprising trimethylopropane divalerate monopalargonate and from 0.25% to 3% by weight of phenyl- $\alpha$ -naphthylamine, and from 0.25% to 3% by weight of nickel bis (N-phenyl-5-nitrosalicylimine).

35. 11. An anti-oxidant composition comprising a diaromatic secondary amine selected from the group consisting of diaryl amines, aryl-alkaryl amines and dialkaryl amines, and a metal chelate represented by the formula:



wherein Y represents a member selected from the group consisting of NO<sub>2</sub> and H; M represents a member selected from the group consisting of Ni, Co, and Zn; R represents a member selected from the group consisting of



and



and X represents a member selected from the group consisting of H, CH<sub>3</sub>, and Cl, the said components being present in a weight ratio of from 0.25:3 to 3:0.25,

12. An anti-oxidant composition comprising phenyl- $\alpha$ -naphthylamine and a metal chelate represented by the formula:



wherein Y represents a member selected from the group consisting of  $\text{NO}_2$  and H; M represents a member selected from the group consisting of Ni, Co, and Zn; R represents a member selected from the group consisting of

15



and



and X represents a member selected from the group consisting of H,  $\text{CH}_3$ , and Cl, the said components being present in a weight ratio of from 0.25:3 to 3:0.25.

13. An anti-oxidant composition comprising phenyl- $\alpha$ -naphthylamine and nickel bis (N-phenyl-5-nitrosalicyli-

mine) in a weight ratio of from 0.25:3 to 3:0.25.

14. An anti-oxidant composition comprising phenyl- $\alpha$ -naphthylamine and nickel bis (N-phenyl-5-nitrosalicyli-

mine) in a weight ratio of from 0.5:2 to 2:0.5.

15. An anti-oxidant composition comprising phenyl- $\alpha$ -naphthylamine and nickel bis (N-phenyl-5-nitrosalicyli-

mine) in equal amounts by weight.

References Cited by the Examiner

UNITED STATES PATENTS

|           |         |         |       |          |
|-----------|---------|---------|-------|----------|
| 2,615,860 | 10/1952 | Burgess | ----- | 260—429  |
| 3,036,005 | 5/1962  | Koch    | ----- | 252—49.6 |

OTHER REFERENCES

- 20 Calvin et al., Journal of the American Chemical Society, vol. 68 (1946), pp. 2267.

Marvel et al., Journal of the American Chemical Society, vol. 80 (1958), p. 832.

- 25 DANIEL E. WYMAN, Primary Examiner.